



US007154370B2

(12) **United States Patent**  
Szwarc et al.

(10) **Patent No.:** US 7,154,370 B2  
(45) **Date of Patent:** Dec. 26, 2006

(54) **HIGH PRECISION POWER RESISTORS**(75) Inventors: **Joseph Szwarc**, Ramat-Gan (IL); **Reuven Goldstein**, Herzlia (IL)(73) Assignee: **Vishay Intertechnology, Inc.**, Malvern, PA (US)

(\* ) Notice: Subject to any disclaimer, the term of this patent is extended or adjusted under 35 U.S.C. 154(b) by 90 days.

(21) Appl. No.: 10/762,609

(22) Filed: Jan. 22, 2004

(65) **Prior Publication Data**

US 2004/0150505 A1 Aug. 5, 2004

**Related U.S. Application Data**

(62) Division of application No. 10/304,261, filed on Nov. 25, 2002, now Pat. No. 6,892,443.

(51) **Int. Cl.****H01C 7/06** (2006.01)(52) **U.S. Cl.** ..... 338/7; 338/9; 338/99; 338/204; 338/320; 29/610.1(58) **Field of Classification Search** ..... 338/59, 338/309, 320, 7, 9, 99, 203, 308; 29/610.1, 29/612, 621

See application file for complete search history.

(56) **References Cited**

## U.S. PATENT DOCUMENTS

3,405,381 A \* 10/1968 Zandman et al. ..... 338/254

|              |   |        |                     |         |
|--------------|---|--------|---------------------|---------|
| 4,318,072 A  | * | 3/1982 | Zandman .....       | 338/7   |
| 4,677,413 A  |   | 6/1987 | Zandman et al.      |         |
| 4,774,491 A  | * | 9/1988 | Vugts .....         | 338/306 |
| 5,039,976 A  |   | 8/1991 | Drabkin             |         |
| 6,194,990 B1 | * | 2/2001 | Lee et al. .....    | 338/320 |
| 6,404,323 B1 | * | 6/2002 | Schrum et al. ..... | 338/92  |
| 6,404,324 B1 | * | 6/2002 | Witt et al. .....   | 338/320 |
| 6,873,028 B1 | * | 3/2005 | Belman .....        | 338/308 |

**OTHER PUBLICATIONS**

New Z-Based Foil Technology Enhances Resistor Performance, Featured Technical Paper, Jul./Aug. 2002, Reaven Goldstein and Joseph Szwarc.

\* cited by examiner

*Primary Examiner*—Tu Hoang(74) *Attorney, Agent, or Firm*—McKee, Voorhees & Sease, P.L.C.

(57)

**ABSTRACT**

A high precision power resistor having the improved property of reduced resistance change due to power is disclosed. The resistor includes a substrate having first and second flat surfaces and having a shape and a composition; a resistive foil having a low TCR of about 0.1 to about 1 ppm/ $^{\circ}$  C. and a thickness of about 0.03 mils to about 0.7 mils cemented to one of the flat surfaces with a cement, the resistive foil having a pattern to produce a desired resistance value, the substrate having a modulus of elasticity of about  $10 \times 10^6$  psi to about  $100 \times 10^6$  psi and a thickness of about 0.5 mils to about 200 mils, the resistive foil, pattern, type and thickness of cement, and substrate being selected to provide a cumulative effect of reduction of resistance change due to power.

**13 Claims, 3 Drawing Sheets**



Fig. 1



Fig. 2



Fig. 3



Fig. 4



Fig. 5



Fig. 6

**1**  
**HIGH PRECISION POWER RESISTORS**

**CROSS-REFERENCE TO RELATED  
APPLICATIONS**

This application is a divisional of and claims priority to U.S. patent application Ser. No. 10/304,261 filed on Nov. 25, 2002 now U.S. Pat. No. 6,892,443.

**BACKGROUND OF THE INVENTION**

It is well known to obtain low TCR (Temperature Coefficient of Resistance) resistors. Said resistors will change very little in their resistance when subject to uniform temperature changes. For example, wirewound or thin film or foil resistors may change as little as 3 ppm/<sup>o</sup> C. In other words, if the ambient temperature changes from 25<sup>o</sup> C. to 125<sup>o</sup> C. (a 100<sup>o</sup> C. temperature difference) the resistor will change (3 ppm/<sup>o</sup> C.) (100<sup>o</sup> C.)=300 ppm  $\Delta R/R$ . The resistor property of low TCR is therefore useful and desirable where high precision is required and ambient temperature changes may occur.

However, if the same resistor is subject to electric power (current) without a change in ambient temperature the resistance can also change several hundred ppm's depending on the power applied. This phenomena is sometimes described as the Joule effect or resistor self-heating. Both resistance changes due to changes in ambient temperature and resistor changes due to electric power phenomena are additive.

For applications where resistors are used as current sensors (i.e. 4 contact devices) such changes in resistance due to self-heating would, in many cases, be so significant so as to make such resistors unsuitable for accurate current sensing. To resolve this problem, one uses several resistors connected in parallel to distribute the heat due to power across the plurality of resistors so that the temperature of each resistor is reduced and the effect of self-heating is reduced. There are significant disadvantages to this approach, however, as the resulting component is larger (several resistors as opposed to a single resistor), more costly in materials, requires labor for assembly, and the component takes up more space on a printed circuit board than a single resistor. Thus, problems remain.

Therefore, it is a primary object of the present invention to improve upon the state of the art.

It is a further object of the present invention to provide a resistor with suitable properties for use as a high precision power resistor.

A still further object of the present invention is to provide a resistor suitable for use in current sensing applications.

Another object of the present invention is to provide a resistor that demonstrates only small changes in resistance due to power.

Yet another object of the present invention is to provide an improved resistor designed to take into account properties of the resistive foil adhesive cement and substrate to provide a cumulative effect of reduction of resistance change due to power.

A further object of the present invention is to provide a resistor that can be manufactured on a large scale and at a reasonable cost.

One or more of these and/or other objects, features, or advantages of the present invention will become apparent from the Specification and claims that follow.

**2**

**SUMMARY OF THE INVENTION**

The present invention provides for a high precision power resistor. The power induced resistance change of the resistor is substantially reduced. To do so, the present invention takes into account construction of the resistor, properties of the cement, the shape and type of substrate, the resistor foil, and the pattern design for the resistor foil.

According to one aspect of the invention, a resistor is provided that includes a substrate having first and second flat surfaces and having a shape and a composition. The resistor also includes a resistive foil having a low TCR of about 0.1 to about 2 ppm/<sup>o</sup> C. and a thickness of about 0.03 mils to about 0.7 mils cemented to one of the flat surfaces of the substrate with the cement. The resistive foil has a pattern to produce a desired resistance value. The substrate also has a modulus of elasticity of about  $10 \times 10^6$  psi to about  $100 \times 10^6$  psi and a thickness of about 0.5 mils to about 200 mils. The resistive foil, pattern, cement and substrate are selected to provide a cumulative effect of reduction of resistance change due to power.

According to another aspect of the present invention, a method for producing a resistor is disclosed. The method includes cementing a first resistive foil and a second resistive foil to opposite surfaces of a substrate, the first and second foils patterned to have approximately equal resistance values, interconnecting the first and second resistive foils to provide approximately equal power dissipation on the first and second surfaces of the substrate, thereby reducing temperature gradients across the substrate, preventing bending of the substrate, and avoiding resistance change due to bending of the substrate.

**BRIEF DESCRIPTION OF THE DRAWINGS**

35 FIG. 1 is a graph showing change in resistance versus temperature for both foil before cementing to a substrate and change in resistance due to stress after cementing the foil to a substrate.

40 FIG. 2 is a graph showing change in resistance versus temperature for the cumulative effect of the foil and the stress after cementing the foil.

45 FIG. 3 is a perspective view of one embodiment of a resistor according to the present invention.

FIG. 4 is a cross-section of one embodiment of a resistor according to the present invention.

FIG. 5 is a diagram showing one embodiment of a foil pattern according to the present invention.

FIG. 6 is a cross-section of the second embodiment of a resistor according to the present invention, illustrating an alternative method of achieving a resistor with a reduced power coefficient of resistance.

**DETAILED DESCRIPTION OF THE  
INVENTION**

55 A resistor with a very low TCR (ambient temperature conditions) can be obtained by using a resistive foil with an inherent TCR such that it essentially balances the  $\Delta R/R$  induced by stress when the foil is cemented to a substrate with a different coefficient of thermal expansion as the foil. The basic phenomena is shown in FIGS. 1 and 2. In addition, relevant discussion is provided in U.S. Pat. No. 4,677,413 to Zandman and Szwarc, herein incorporated by reference in its entirety.

60 FIG. 1 provides a graph showing a change in resistance versus temperature for both foil before cementing to a

substrate 14 and change in resistance due to stress after cementing the foil to a substrate 16. As shown in FIG. 1, the temperature axis 10 and the  $\Delta R/R$  axis 12 are shown. The curve 14 represents change in resistance versus temperature for the foil before cementing to a substrate. As shown, the change in resistance increases in a nonlinear fashion as a function of temperature. The linear relationship 16 is also shown for changes in resistance due to stress after the foil has been cemented to a substrate. As shown in FIG. 1, as the temperature increases, the resistance decreases. Both the changes in resistance of the foil and changes in resistance due to stress occur simultaneously when temperature changes.

FIG. 2 is a graph showing change in resistance versus temperature for the cumulative effect of the foil and the stress after cementing the foil to the substrate. In FIG. 2, the cumulative effect is indicated by reference numeral 18. The effect of the change in resistance due to temperature changes of the foil and the change in resistance due to stress after cementing the foil to the substrate are offsetting to some degree. Thus, the resulting effects can be used to decrease the resistance changes due to temperature changes. In particular note the area near the crossing of axis 12 and 10 is relatively flat and close to 0. Complete zero is very difficult to obtain because of non-linearity of curve 14 in FIG. 1.

A resistor with a very low TCR can be obtained with many types of foil, many substrate thicknesses, many substrate materials, many types of cements and cement thickness, however such a resistor will show substantial changes in resistance when subject to electric power as opposed to only ambient temperature changes. However, if the cement type and thickness, foil type and its inherent TCR and substrate type and shape and the geometry of pattern of the foil resistive element are chosen very carefully the power induced resistance change can be reduced very substantially as discovered herein.

What the present inventors have discovered is the ability to substantially influence resistance change due to power by the selection of the cement, shape and type of substrate and pattern design of the resistor foil. When power is applied to the foil it produces a higher temperature than the one in the substrate. This temperature differential across the thickness of substrate produces bending in the substrate. Such bending amount also depends on the heat transmissivity of the cement and the cement's thickness. Furthermore, if the pattern is made with longitudinal and transverse strands the strain induced by bending can be decreased by the strain effect of Poisson's ratio in certain shapes of substrate depending on it's ratio of width to thickness. Poisson's ratio is the ratio of longitudinal strain to transverse strain.

The inventors have discovered that if a proper balance is made to account for all these factors a resistor can be constructed which will show a much better performance than other power resistors. The resistor can get hot and yet it will show only very small changes in resistance due to power. This is a very significant advantage over prior art resistors.

FIGS. 3 through 5 illustrate one resistor according to the present invention. FIG. 3 illustrates resistor 20. The resistor 20 includes an alumina substrate 22 having a length, a width, and a thickness. A resistive foil 26 of Ni/Cr of 0.100 mils in thickness and having a TCR of 0.2 ppm/ $^{\circ}$  C. is cemented to the substrate 22 with an epoxy cement 24 having a modulus of elasticity of 450,000 psi and a thickness of 0.5 mils. When subject to one watt power, the resistor has a change in resistance of less than 30 ppm. The same type resistor under

same conditions where the cement is of different thickness, and the TCR is 2 ppm/ $^{\circ}$  C., will change resistance by 300 ppm or more.

The substrate 22 of the resistor 20 has first and second flat surfaces. The substrate has a shape and a material composition. The resistive foil preferably has a thickness of about 0.03 mils to about 0.5 mils and a TCR of about 0.1 to about 1 ppm/ $^{\circ}$  C. when cemented to one of the flat surfaces with a cement. The resistive foil 26 has a pattern selected to produce a desired resistance value. The foil pattern can be made with longitudinal and transverse strands. The substrate 22 preferably has a modulus of elasticity of about  $10 \times 10^6$  psi to about  $100 \times 10^6$  psi and a thickness of about 0.5 mils to about 200 mils. The resistive foil, pattern, cement and substrate being chosen to provide a cumulative effect of reduction of resistance change due to power. The parameters are preferably chosen so that the resistance change of the resistor due to power will only be a small fraction (25% or less) of what it would have changed if the same resistance foil was used but it was with a TCR of more than 1 ppm/ $^{\circ}$  C. and cemented to the substrate with different geometric and physical characteristics of the cement, pattern and substrate.

The parameters such as the shape of the substrate, the composition of the substrate, the thickness of the substrate, the TCR of the resistive foil, the type of cement, the heat transmissivity of the cement, and the thickness of the cement are also preferably selected to provide the cumulative effect of reduction of resistance change due to power.

It is to be understood that further assembly of the resistor 20 will proceed in accordance with techniques which are generally known in the art. Such subsequent steps could include connecting leads or contacts (not shown), adding protective materials, or other known steps that may be appropriate for a particular application.

The present invention contemplates that other types of substrates can be used of various shape compositions and thicknesses. The composition of alumina is simply one convenient type of substrate. Similarly, the resistance foil can be of any number of materials. Ni/Cr is simply one common and expedient selection. The present invention also contemplates that various types of cement, epoxy or otherwise, can also be used.

A second embodiment of the present invention is illustrated in FIG. 6. Here the resistor 30 is constructed such that foil 36 is cemented on a first surface of the substrate 32 and a second resistive foil 37 on an opposite surface of the substrate 32.

The two foils (36 and 37) are etched in a pattern forming similar or approximately equal resistance values and are interconnected, in parallel or in series. When power is applied to the resistor, the two opposite surfaces are heated equally. This results in a minimal heat flow across the substrate as there is no temperature differential across the substrate's thickness and its bending is prevented. This second embodiment of FIG. 6 involves higher manufacturing costs compared to the first embodiment. Thus, a high precision power resistor has been disclosed that provides advantages over the state of the art.

What is claimed is:

1. A resistor comprising:  
an insulating substrate having first and second opposite flat surfaces and having a shape and a composition;  
a first resistive foil having a low TCR of 0.1 to 1 ppm/ $^{\circ}$  C. and a thickness of 0.03 mils to about 0.7 mils cemented to the first flat surface with a cement;

a second resistive foil having a low TCR of 0.1 to 1 ppm/<sup>o</sup> C. and a thickness of 0.03 mils to 0.7 mils cemented to the second flat surface, the second resistive foil connected to the first resistive foil, the first resistive foil and second resistive foil having approximately equal resistance values and providing approximately equal power dissipation on both surfaces of the substrate thereby reducing temperature gradients across the substrate, preventing bending of the insulating substrate, and avoiding resistance change associated with bending;

the insulating substrate having a modulus of elasticity of  $10 \times 10^6$  psi to  $100 \times 10^6$  psi and a thickness of 0.5 mils to 200 mils;

the first and second resistive foil each having a pattern to produce a desired resistance value;

the insulating substrate, the first resistive foil, the second resistive foil and each pattern being selected to provide a cumulative effect of reduction of resistance change due to power.

2. The resistor of claim 1 wherein the shape of the insulating substrate is selected to provide the cumulative effect of reduction of resistance change due to power.

3. The resistor of claim 1 wherein the composition of the insulating substrate is selected to provide the cumulative effect of reduction of resistance change due to power.

4. The resistor of claim 1 wherein the thickness of the insulating substrate is selected to provide the cumulative effect of reduction of resistance change due to power.

5. The resistor of claim 1 wherein the TCR of the first resistive foil and the TCR of the second resistive foil are selected to provide the cumulative effect of reduction of resistance change due to power.

6. The resistor of claim 5 wherein each of the first and second resistive foils is etched to form longitudinal and transverse strands in patterns selected to reduce bending and provide the cumulative effect of reduction of resistance change due to applied power.

7. The resistor of claim 1 wherein the cement is selected to provide the cumulative to reduce the effect of resistance change due to power.

8. The resistor of claim 6 wherein the heat transmissivity of the cement is selected to provide the cumulative effect of reduction of resistance change due to power.

9. The resistor of claim 6 wherein the thickness of the cement is selected to provide the cumulative effect of reduction of resistance change due to power.

10. The resistor of claim 1 wherein the TCR is determined for a temperature range from 25° C. to 125° C.

11. The resistor of claim 1 wherein the first and second resistive foil, each pattern, and the insulating substrate are selected to provide the cumulative effect of reduction of resistance change due to power by offsetting change in resistance due to temperature changes in the first and second resistive foils with change in resistance due to stress after cementing the first and second resistive foils to the substrate.

12. The resistor of claim 1 wherein an operating temperature for the resistor is greater tan ambient temperature.

13. A power resistor, comprising:  
an insulating substrate having first and second opposite flat surfaces and having a shape and a composition;  
a first resistive foil having a low TCR of 0.1 to 1 ppm/<sup>o</sup> C. and a thickness of 0.03 mils to about 0.7 mils cemented to the first flat surface with a cement;

a second resistive foil having a low TCR of 0.1 to 1 ppm/<sup>o</sup> C. and a thickness of 0.03 mils to 0.7 mils cemented to the second flat surface, the second resistive foil connected to the first resistive foil, the first resistive foil and second resistive foil having approximately equal resistance values and providing approximately equal power dissipation on both surfaces of the substrate thereby reducing temperature gradients across the substrate, preventing bending of the insulating substrate, and avoiding resistance change associated wit bending;

the insulating substrate having a modulus of elasticity of  $10 \times 10^6$  psi to  $100 \times 10^6$  psi and a thickness of 0.5 mils to 200 mils;

the first resistive foil, the second resistive foil, and insu-

lating substrate being selected to provide a cumulative

effect of reduction of resistance change due to power;

and  
wherein the shape of the insulating substrate, the compo-

sition of the insulating substrate, and the TCR of the

first resistive foil are selected to provide the cumulative

effect of reduction of resistance change due to power.

\* \* \* \* \*

UNITED STATES PATENT AND TRADEMARK OFFICE  
**CERTIFICATE OF CORRECTION**

PATENT NO. : 7,154,370 B2  
APPLICATION NO. : 10/762609  
DATED : December 26, 2006  
INVENTOR(S) : Szwarc et al.

Page 1 of 1

It is certified that error appears in the above-identified patent and that said Letters Patent is hereby corrected as shown below:

Col. 6, Claim 12, line 14:

After "greater" delete "tan" and add -- than --

Signed and Sealed this

Sixth Day of March, 2007

A handwritten signature in black ink, appearing to read "Jon W. Dudas". The signature is written in a cursive style with a large, stylized 'J' and 'W'.

JON W. DUDAS  
*Director of the United States Patent and Trademark Office*